

Oct. 4, 1932.

P. DREWSSEN

1,880,899

PROCESS OF MANUFACTURING STRAW PAPER

Filed Oct. 13, 1930



## UNITED STATES PATENT OFFICE

PIERRE DREWSSEN, OF SANDUSKY, OHIO, ASSIGNOR TO THE HINDE & DAUCH PAPER COMPANY, OF SANDUSKY, OHIO, A CORPORATION OF OHIO

## PROCESS OF MANUFACTURING STRAW PAPER

Application filed October 13, 1930. Serial No. 488,493.

The invention relates to the manufacture of straw paper and more particularly to that type used in the manufacture of corrugated wrappers and shipping containers. It is the 5 object of the present invention to simplify the process by the elimination of one step heretofore used as well as the apparatus required therefor. It is a further object to shorten the time required in treatment and 10 to obtain a product having properties equal or superior to those of the product produced by the usual method. With these objects in view the invention consists in the construction as hereinafter set forth.

15 The drawing is a diagrammatic representation or flow sheet indicating the successive steps of my improved process.

In the present state of the art the method of manufacture of straw paper consists of three 20 principal operations: First, the wheat, rye, oat or other straw is cooked in rotary digesters with alkali and water. Various formulas are used, some of them being approximately 5% lime and 5% soda ash based on the dry 25 weight of the straw; or 10 to 14% high calcium lime based on the dry weight of the straw; or a mixture of caustic soda and sulphide of soda, the total chemicals used being about 4 to 7% based on the dry weight of the straw.

30 The steam pressure used varies from 15 to 60 pounds per square inch and the time of cooking from 6 to 10 hours, or over night, and about two or three pounds of water are used per pound of dry straw in the rotary digester.

35 The second operation consists in beating the cooked straw and jordaning the same in order to draw out the fibres and reduce their length to make them suitable for the paper machine.

40 During the beating operation the general practice is to wash the stock in order to remove as much of the spent cooking liquor as possible. The third operation consists in forming the beaten and jordaned fibres into

45 a sheet on the paper machine according to the well known art in which cylinder or Fourdrinier paper machines are used.

The rotary digesters used in the first operation hold approximately 14,000 pounds of dry straw per charge, but in order to intro-

duce this quantity it is necessary to fill the rotaries with successive amounts of straw, each of which must be wilted down separately. For example, approximately 6,000 pounds of straw are introduced during the 55 first fill together with the water and cooking chemicals. The cover is then put on and the rotary is cooked for about one hour, more or less. The steam pressure is then blown down and an additional quantity of straw is introduced. The cover is then put on again and the charge is cooked for approximately 60 one hour more. The steam pressure is then blown off and a further quantity of straw introduced, and so on, for about five or six 65 fills during the course of which a total of about 14,000 pounds of straw are introduced, provided there are enough rotaries available to prepare sufficient stock for a 24 hour run on the paper machine. In this case the introduction of this straw requires approximately a whole working day, consequently it becomes necessary to cook the rotaries all 70 night and to blow them down and empty them early in the morning. For a mill making sixty or seventy tons of straw paper in twenty-four hours, it is necessary to have about sixteen or more rotary digesters available. This involves a considerable capital 75 investment in digesters including drives for same, foundations, conveyors, buildings to house them, etc., and it also involves the labor of nine or ten men in order to fill, empty and cook these digesters, as well as to handle the cooked straw.

In some mills however, there are not enough rotary digesters for one cook each per 80 24 hours. Where this is the case it is necessary to operate on as few as three fills of straw twice in 24 hours instead of on six fills 85 once in 24 hours. This makes it necessary to approximately double the number of rotary house operators to supply enough cooked straw material to keep up with the demand of the paper machine.

In some mills it is the practice to empty the rotaries on a conveyor which heaps the cooked straw in a seasoning room from which it is manually forked or shovelled to another conveyor which brings it into the beater 90 100

room. The object of this seasoning is to soften the straw still further and to bring about a certain mixing of stock from different rotaries.

5 Whether there are sufficient rotaries or not, the filling of these rotaries with straw presents a problem which is caused by the bulky, nature of dry, baled straw and the length of time it takes to wilt it down to a smaller 10 volume. In present practice this problem is met by employing a comparatively large number of men to stuff in the straw and by using a large number of rotaries to wilt it down during the period allotted for this 15 purpose.

15 By means of the process which I shall outline below, I have found it possible to eliminate the entire first operation mentioned above, namely, the use of rotary digesters in 20 the manufacture of straw paper for corrugated boxes. I have found that it is possible and practicable to reduce and wilt raw, dry straw in the presence of hot water and caustic alkali in a paper mill beater of the ordinary 25 type. Approximately 10% alkali, more or less, based on the dry weight of the straw is added to the batch together with about 20 pounds of water per pound of straw. The 30 addition of straw to a beater is not essentially different from the addition of pulp or paper stock, but it is essential in this process that the water in the beater be maintained at as high a temperature as possible, say 180 to 205 degrees Fahrenheit, and that caustic 35 alkali be added. The length of time necessary in the beater is approximately one to two hours depending upon the water temperature and the efficiency of the beater. Substantially dry, baled straw wilts down almost 40 immediately under these conditions.

45 After the stock has been treated in beaters for this length of time I find it desirable, in the interest of economy, in order to conserve heat and chemicals, to effect as complete a separation of the hot caustic liquor from the straw substance as possible, and to return the hot caustic liquor to a storage tank from which it may be re-used in the beaters to treat additional quantities of straw, after which 50 additional caustic alkali is added to this liquor to bring it up to the desired strength. An Oliver filter or a Decker or any similar device may be used for this purpose. The amount of caustic to add to the re-used liquor 55 can be determined by a simple calculation based on titrating a known amount of this liquor with a standard acid solution using a suitable indicator, such as phenolphthalein, which anyone skilled in the practice of analytical chemical methods will understand.

60 The separation of the beaten stock from the caustic liquor may be made more complete by spraying the filtered fiber with water while still on the cylinder mould of the Oliver, 65 this wash water being combined with the

filtered caustic liquor in such proportion that the total volume of caustic liquor in circulation remains approximately constant.

The separated straw stock may then be treated still further in beaters, or it may be passed directly to the Jordan engines from which it reaches the Fourdrinier or cylinder paper machine where the paper is formed, dried and calendered. This stock will necessarily contain some residual caustic, the presence of which may be injurious to the wool felts of the paper machine. I find it desirable to neutralize at least a portion of this residual alkalinity to the point where the felts will be protected, by adding a stream of acid substance at the head box, vat or receiver of the paper machine. Sulphuric acid, if carefully controlled, sulphurous acid, sulphate of alumina, sulphate of iron, nitre cake or any suitable acid material may be used for this 85 purpose. In fact it is not necessary to neutralize this alkalinity to as low a pH as 7.0, since experience demonstrates that a pH of 8.0 or higher may be used on the machine wire without damage to the blankets or the paper product. In fact, the more alkaline the stock is at the paper machine wire, the higher will be the crushing resistance of the corrugations in the finished corrugated sheet.

90 As diagrammatically represented in the drawing the straw from stacks or other source of supply A is weighed on scales B and fed into a large breaker or beater tank C. The caustic received from a source D is first introduced into a tank E and through a 100 measuring tank F into the beater tank C. If lime is used in the treatment, it is introduced from bags into the tank C. After treatment in the tank C the material passes to the filter G in which the partially defibered pulp is separated from the caustic liquor, the latter passing to a tank H from which it is returned to the tank C. The pulp is passed on to a chest I from which it is introduced into the secondary beaters J J', thence to the chest K, to the Jordan L and screen M to the head box or vat N of the paper machine O. Neutralization is effected by an acid substance supplied from the tank P and introduced into the vat N.

105 In addition to the advantages incident to the elimination of rotary digester cooking, the cost of additional men, and other financial "overhead", the above described process produces a sheet of straw paper which is considerably superior to those made by present methods, and in addition to this, my improved process offers a more simple but vastly more efficient means of control of both process and quality of finished product.

110 If, for example, it is desired to manufacture a sheet of corrugated paper where a combination of extreme lightness of weight and great crushing resistance are essential, such paper can be produced merely by maintaining a slightly higher concentration of caustic 115

soda, but no lime, in the hot water in the beaters. On the other hand, if a somewhat more bulky sheet of greater weight but lower strength is desired, as for instance for the so-called egg case filler, in other words, the 5 soft yellow partitions frequently used to create individual compartments for eggs in shipping containers, or if a soft grade of corrugating paper is desired where high crushing resistance is not imperative, such paper 10 can be made by eliminating the use of caustic soda entirely and using in its place approximately ten per cent of high calcium lime, based on the dry weight of the straw. Again, if a paper of strength somewhere between 15 these extremes is desired, a mixture of say five per cent caustic soda and five per cent caustic high calcium lime may be used in the hot water in the beaters. Still another variation 20 in my process would be to use varying mixtures of caustic high calcium lime and soda ash, the interaction of which would produce caustic soda and calcium carbonate, and if an excess of lime were used, the straw 25 would in this case be acted upon by caustic lime and caustic soda. One possible disadvantage of this variation for certain purposes would be the presence of insoluble carbonate which might reduce the strength of the sheet; also the presence of carbonates may cause 30 foaming if acid substances are used to neutralize excess alkalinity, as mentioned above.

Still another variation to this process 35 would be to increase or reduce the quantity of caustic soda above or below ten per cent, based on the dry weight of the straw, without using any lime at all. An increase in caustic soda tends to hydrate the straw substance still further and thereby to increase 40 the moisture content of the sheet at the dryers of the paper machine which, while it results in reduced paper production, increases the strength of the paper. A reduction in the concentration of caustic soda in the beaters 45 to say seven per cent results in a greater power consumption but produces a fibrous stock which separates from its water of suspension more readily on the wire of the paper machine. This property tends to increase 50 the production of paper, which, however, has a lesser strength.

While it is impossible to state definitely 55 any fixed limits of crushing resistance of corrugated papers made by this process, on account of the natural variations produced by equipment differences and lack of uniformity of operating conditions among straw paper mills, nevertheless the following may give some idea of the said limits.

If 10% of high calcium caustic lime (CaO) 60 based on the weight of the dry raw straw is used in the beater without any caustic soda (NaOH), a sheet of straw paper which weighs approximately 36 pounds per 1000 65 square feet will, when corrugated on a reg-

ular Langston type corrugator of about three .175 inch arches per linear inch, produce a corrugated product which has a strength of about 200 Webb units. If 10% caustic soda without any lime, based on the weight of the 70 raw dry straw, is used in the beater, a sheet of paper weighing only about 28 pounds per 1000 square feet, similarly corrugated, will yield to crushing under a force of 350 Webb units more or less. The former sheet of 200 75 Webb units is comparable in strength with rotary cooked paper where lime alone has been used, whereas the 350 Webb unit paper is superior in strength to a sheet made from rotary cooked straw where caustic soda or 80 lime-soda ash mixture has been used. Such rotary-lime-soda ash sheets seldom exceed 300 Webb units even when they weigh 34 pounds per 1000 square feet. The superiority 85 of this improved paper in strength and weight is therefore obvious, and the improved control of manufacturing operations is evident.

In straw paper mills it is frequently the custom to utilize box board clippings, old 90 papers, folded news, etc., as fibrous material which is mixed with the straw fiber to a certain limited extent. In the above description process and variations of the same, old papers may be similarly admixed, although 95 such blending tends to defeat one of the objects of this invention, namely, the production of a light, strong sheet.

What I claim as my invention is:

1. In the process of manufacturing straw 100 paper, the step of simultaneously treating the straw with alkali and beating to separate the same into fibre bundles.
2. In the process of manufacturing straw 105 paper, the step of introducing dry straw into a hot alkali bath and simultaneously beating to separate the same into fibre bundles.
3. In the process of manufacturing straw 110 paper, the introduction of the dry straw into a bath of caustic alkali, mechanically disintegrating the straw while in said bath to separate the same into fibre bundles, separating a portion of the alkali solution with its dissolved impurities from the pulp and 115 re-using the impure alkali solution for the treatment of additional straw.

4. In the process of manufacturing straw 120 paper, the step of mechanically disintegrating the straw into fibre bundles in the presence of from seven to twelve per cent caustic alkali based on the dry weight of the straw.

5. In the process of manufacturing straw 125 paper, the step of passing the straw successively between beaters in the presence of hot water containing from seven to twelve per cent of caustic alkali based on the dry weight of the straw.

6. In the process of manufacturing straw 130 paper, the step of separating the straw into

fibre bundles in the presence of water heated from 150 degrees to 212 degrees Fahrenheit and containing from seven to twelve per cent caustic alkali.

7. In the process of manufacturing straw paper, the step of partially neutralizing the alkalinity of the straw to a pH test of 8.0 or higher by the addition of acid.

8. In the process of manufacturing straw paper including the beating of the straw 10 in the presence of caustic alkali, the step of filtering the partially defibered pulp from the partly exhausted alkaline liquor and returning the latter together with dissolved impurities for further use.

15 9. In the process of manufacturing paper from straw, the step which consists in wilting the straw continuously and rapidly in a breaker beater.

10. In the process of manufacturing paper 20 from straw, the step of wilting the straw continuously and rapidly in a hot aqueous alkaline mixture in a breaker beater.

11. In the process of manufacturing paper 25 from straw, the step which consists of treating substantially raw dry straw in a breaker beater with black liquor from an alkaline process.

In testimony whereof I affix my signature.

30 PIERRE DREWSSEN.